

Aug. 19, 1941.

R. M. EVANS

2,253,070

COLOR CORRECTION IN PRINTING MULTILAYER FILM

Filed Aug. 16, 1940



RALPH M. EVANS  
INVENTOR

BY *Newton M. Penning*  
*R. Frank Smith*  
ATTORNEYS

## UNITED STATES PATENT OFFICE

2,253,070

## COLOR CORRECTION IN PRINTING MULTI-LAYER FILM

Ralph M. Evans, Rochester, N. Y., assignor to  
Eastman Kodak Company, Rochester, N. Y., a  
corporation of New Jersey

Application August 16, 1940, Serial No. 352,902

4 Claims. (Cl. 95—2)

This invention relates to printing multi-layer color film and particularly to a method for obtaining color correction in printing such film.

It is well known that color prints made by uncorrected methods of photographic color reproduction suffer from degradation with more or less gray. This is due to the fact that some of the pigments or dyes used in the color print absorb light not only in the spectral regions which they are intended to absorb but also to some extent in other regions. According to the subtractive method of color photography, the color separation images are printed in colors complementary to the colors of the taking filters or the sensitivity of the emulsion layers. In three-color photography the primary colors are considered to be red, green and blue and the color separation images obtained from these are printed respectively in blue-green, magenta and yellow colors. If theoretically accurate dyes could be obtained, these dyes should absorb only their complementary colors. The blue-green should absorb the red region of the spectrum and transmit the blue and the green regions. Similarly, the magenta dye should absorb the green region of the spectrum and transmit the blue and the red regions, and the yellow dye should absorb the blue region and transmit the red and the green regions.

Dyes have not yet been found for use in color photography which absorb only in the proper spectral regions. The blue-green dye usually absorbs not only in the red region but also to some extent in the green and the blue regions. The magenta dye absorbs not only in the green region but also in the blue and red regions. The yellow dye, on the other hand, is usually quite efficient, absorbing very little except in the blue and violet region.

As a result of the light absorption of the blue-green dye in the blue and green regions of the spectrum, certain corrections must be applied in printing, or a lower concentration of magenta or yellow dye must be used in the print in order to maintain a balance of color in the scale of grays. By using less magenta or yellow dye in the print than would otherwise be used, the gray scale balance is maintained by the blue-greens. Greens and blues of the print are degraded with gray and, therefore, are less luminous than they should be, while magentas, yellows and reds are lacking in saturation, that is, are diluted by white.

In the preparation of color separation negatives or positives by printing from a colored orig-

inal, such as a multi-color transparency, this degradation of colors may be overcome by the use of masks, that is, thin positives in the case of color separation negatives, which are registered with the color separation negative in making the print. When printing from a multi-color image on photographic film onto a similar multi-layer film, it is, of course, impossible to use separate masks for the different color separation records since they must be printed simultaneously onto the printing material. If a single mask is used, the registration difficulties are considerable and in the case of small sized film, such as motion picture film, render this method of color correction impracticable.

I have discovered a method of color correction which is suitable for printing a multi-color image on multi-layer film onto a similar material and also in printing onto separate emulsion layers for making color separation records. It is of special utility in duplicating natural color transparencies or natural color motion picture film.

According to this method an emulsion layer is coated integrally with the multi-layer film prior to exposure and is so treated that a negative image can be printed in it after processing the film to a colored image.

In the accompanying drawing a series of sectional views shows the steps in the method of preparing a printing element according to my invention.

The usual type of multi-layer film consists of a support having coated thereon three emulsion layers effectively sensitive respectively to the red, green and blue regions of the spectrum. My invention consists in coating as a top or outer layer on a film of this type a thin emulsion layer which has been fogged prior to coating or which is fogged in a suitable manner after coating so that it will be developed in a silver halide developer when the film is developed. In this layer a low contrast negative is made after the film has been processed to colored images and this negative silver image serves as a mask in printing the colored image. In a suitable manner hereinafter described the masking layer is made color-sensitive, usually red-sensitive, since it is ordinarily desired to correct the deficiency in the spectral transmission in this region of the blue-green and magenta dyes used in reproduction. This layer may be sensitized to other regions of the spectrum if correction in other ways is desirable. The layer may be sensitized so that it may be partly exposed to light of one color and partly to light of another color. According to

the desired form of the process, however, the masking layer is made sensitive to red light after color processing of the film and the film is then exposed through the support with red light so that those portions of the color picture which transmit red light are recorded on the masking layer as darker than those portions which absorb red light. Thus, in addition to recording the natural red light transmission of the yellow and magenta dyes, the red light transmission of the blue-green dye is also recorded on the masking layer.

Although my process may be used in any color method in which a multi-layer element is processed so that no image is formed in the masking layer prior to the development of the masking image, my process has been designed for use with a method such as that described in Mannes, Godowsky and Wilder U. S. patent application Serial No. 185,700, filed January 19, 1938. According to the method described in that application, a multi-layer photographic element consisting of three emulsion layers sensitized respectively to the red, green and blue regions of the spectrum are coated on one side of a single support. After exposure and negative development of this film, the emulsion layers are selectively fogged and colored images are formed therein. After negative development, the bottom red-sensitive emulsion layer is exposed through the support to red light and the film is then developed in a blue-green color forming developer which produces a blue-green positive image in the bottom layer. Similarly, the top layer is exposed from the outer side and is developed in a yellow color forming developer which produces a yellow positive image in the top layer. The middle layer may then be exposed or otherwise fogged as by the use of suitable chemical fogging agents to render the residual silver halide in that layer developable after which the film is again developed in a color forming developer to produce a magenta positive image in the middle layer.

According to the present invention the masking layer which has been fogged prior to the first development of the film is developed to a uniform silver image in the first or negative developer and remains in this form during color processing of the film. In the normal processing of a photographic element of this type after colored images are formed in the emulsion layers and silver negative and positive images still remain, these silver images are removed by converting them to a soluble silver salt which is then removed in hypo. This step is modified according to my invention by converting the silver in the masking layer to silver halide and then sensitizing the silver halide in this layer to red light by bathing in a suitable sensitizing bath. Before this red sensitization of the masking layer, the silver images in the lower three layers are removed in a bath which does not affect silver halide. Because of the removal of silver from the layers containing the colored images, these layers are no longer sensitive. A printing exposure may, therefore, be given through the support, that is, through the colored images, onto the red sensitive masking layer using red light for the exposure. This red light exposure impresses an image of the red transmission of the image dyes on the masking layer and the film is then developed in an ordinary silver halide developer to produce a silver image in the masking layer. The silver halide in the masking layer can then be removed in hypo, leaving pure dye images in

the emulsion layers and a silver masking image in the top layer. This film may then be used for printing onto a multi-layer element or for the preparation of color separation images.

5 A specific method of carrying out my process will now be described.

A sensitive element such as that shown in the first stage of the drawing is used consisting of a support 10 of transparent material such as glass, cellulose nitrate, cellulose acetate or other organic acid ester or suitable synthetic resin coated with silver halide emulsion layers 11, 12 and 13 sensitive respectively to the red, green and blue regions of the spectrum. A yellow filter layer 15 (not shown) is incorporated between layers 12 and 13 to prevent the exposure of layers 11 and 12 to blue light in the usual manner. A layer 14 consisting of an ordinary blue-sensitive gelatinous silver halide emulsion is coated over the layer 13. The emulsion comprising the layer 14 is fogged either by light or chemically, preferably prior to coating.

After exposure in a camera or in a printer in the usual way, the film is developed in an ordinary black and white developer. If the film has been properly exposed, development for ten minutes at 20 C. in a developer of the following composition is satisfactory:

|                                    | Grams |
|------------------------------------|-------|
| 30 Monomethyl-p-aminophenolsulfate | 6     |
| Hydroquinone                       | 10    |
| Sodium sulfite                     | 50    |
| Sodium carbonate                   | 30    |
| Potassium bromide                  | 5     |
| 35 Potassium thiocyanate           | 0.5   |
| Water to 1000 cc.                  |       |

This development produces negative silver images 15, 16 and 17 in emulsion layers 11, 12 and 13 and a uniform silver deposit 18 in layer 14, as shown in the second stage of the drawing. The film is then developed as described in application Serial No. 185,700 to form colored images in the emulsion layers but the silver is not bleached or removed in the manner described in that application. The film then contains a blue-green and silver image 19 in layer 11, a magenta and silver image 20 in layer 12, and a yellow and silver image 21 in layer 13 as shown in the third stage of the drawing. The layer 18 is not affected by this treatment and remains in the form in which it existed as shown in the second stage of the drawing.

The next step is the conversion of the silver in the masking layer only, to silver halide. This is accomplished by treating for 2 minutes in a solution which may have the following composition:

|                      |       |     |
|----------------------|-------|-----|
| Quinone              | grams | 2   |
| 60 Potassium bromide | do    | 10  |
| Sulfuric acid        | cc    | 2   |
| Ethyl alcohol        | cc    | 10  |
| Ethylene glycol      | cc    | 850 |
| Water to 1 liter.    |       |     |

65 After rehalogenization of the silver in the top layer 14, the silver in image layers 11, 12, and 13 is then removed. This is done by using an oxidizing bleach bath which does not affect the silver halide in the layer 14, a suitable bath being the following:

|                      |       |   |
|----------------------|-------|---|
| Potassium bichromate | grams | 4 |
| Sulfuric acid        | cc    | 4 |

This bleach is permitted to act for about 6 minutes.

The silver halide in the top layer 14 is then sensitized to red light by bathing for 2 minutes in a solution of the following composition:

|                   |       |       |
|-------------------|-------|-------|
| Pinacyanol        | grams | 0.008 |
| Pyridine          | cc    | 1     |
| Methyl alcohol    | cc    | 75    |
| Benzotriazole     | grams | 1     |
| Water to 1 liter. |       |       |

The film then exists in the form shown in the fourth stage of the drawing, in which there is a blue-green dye image 22 in layer 11, a magenta dye image 23 in layer 12, and a yellow dye image 24 in layer 13. Layer 14 contains a red-sensitive uniform silver deposit 25.

The film is next exposed through the support for about 2 to 3 minutes with red light, such as that transmitted by a Wratten No. 23 or 25 filter. This exposure impresses the red transmission of all of the image forming dyes on the red sensitive silver halide in the top layer 14.

The film is then developed in a black and white developer such as that used in the negative development of the film. This produces a silver masking image 26 as shown in the fifth stage of the drawing. The film is then fixed for about four minutes in hypo, washed for several minutes and dried in warm air. The film then appears as shown in the fifth stage of the drawing with pure dye images 22, 23 and 24 colored respectively blue-green, magenta and yellow in the layers 11, 12 and 13 and silver image 26 in the layer 14. The film is then ready for use in printing onto suitable color sensitive material.

In printing, the masking layer has the effect of increasing the density of the original locally by an amount in approximate inverse proportion to the density of the original to red light. Hence the densities of the whites, magentas, yellows, reds and other colors having a low density to red light are increased most. The density of the blue-greens, blues and greens which have a high density to red light are increased least. Consequently the highlight density of the original is increased and the density range and gamma are reduced. There is, however, no alteration in hue of any portion since the negative mask is neutral gray silver. Only the densities of various portions are increased, and, since the densities of the blues and greens are increased least, these colors appear relative more luminous.

In addition to the use of silver in the mask, it might be made of dye by any suitable method such as by a color forming development. If it is desired to use the original for viewing subsequent to printing, the mask may be removed without damage to the original image. If the mask is of silver, a simple bleaching in ferricyanide and hypo is required and if it is composed of dye it may be removed by a differential

depth bleach such as those described in Mannes and Godowsky U. S. Patent 2,059,887.

In addition to the specific method described, modifications may be made in my process within the scope of the appended claims.

I claim:

1. The method of preparing a multi-color printing element affording corrected color prints, which comprises exposing to an object to be photographed an element having a plurality of superposed emulsion layers sensitive to different spectral regions and an outer, fogged silver halide layer, developing silver images in all said layers including a uniform silver deposit in said

15 outer layer, forming dye and silver images in said differently-sensitive layers, converting the silver in said outer layer only, to silver halide, removing the silver from said differently-sensitive layers, sensitizing the silver halide in said outer layer to 20 a spectral region other than the blue, exposing said outer layer to light of that color through the dye images in the remaining layers, developing a silver image in said outer layer, and removing the silver halide from the outer layer.

2. The method of preparing a multi-color printing element affording corrected color prints, which comprises exposing to an object to be photographed an element having three superposed emulsion layers sensitive to different spectral regions and an outer, fogged silver halide layer, developing silver images in all said layers including a uniform silver deposit in said outer layer, forming positive dye and silver images in said differently sensitive layers by successive

30 color-forming development steps converting the silver in said outer layer only, to silver halide, removing the silver from said differently-sensitive layers, sensitizing the silver halide in said outer layer to red light, exposing said outer layer to red light through the dye images in the remaining layers, developing a silver image in said outer layer, and removing the silver halide from the outer layer.

3. In a method of forming a masked multi-color film having an integral, outer, masking layer, the steps which comprise sensitizing the masking layer to a spectral region other than blue after the formation of colored images in emulsion layers of the film, and printing the mask with light of the color to which the masking layer has been sensitized through said colored images.

4. In a method of forming a masked multi-color film having an integral, outer, masking layer, the step which comprise sensitizing the masking layer to red light after the formation of colored images in emulsion layers of the film, and printing the mask with red light through said colored images.

RALPH M. EVANS.